

1

3,518,195

**CORROSION-INHIBITED AND STABILIZED  
PERFLUORINATED POLYETHER OILS**

Bruce H. Garth, Newark, Del., assignor to E. I. du Pont de Nemours and Company, Wilmington, Del., a corporation of Delaware  
No Drawing. Filed June 5, 1968, Ser. No. 734,571  
Int. Cl. C10m 1/32

U.S. CL. 252—51.5

6 Claims

**ABSTRACT OF THE DISCLOSURE**

Corrosion- and degradation-inhibited oil compositions comprising a perfluorinated polyether oil and a substituted guanamine of the structure



where  $R_f$  is perfluoroalkyl and  $m$  is an integer.

**BACKGROUND OF THE INVENTION**

**Field of the invention**

This invention relates to stabilized perfluorinated polyether oils. More particularly, the invention is directed to such oils containing sufficient amounts of perfluoro-oxo or perfluoropolyoxo- alkane substituted guanamine additives to inhibit corrosion and oil degradation.

**Description of the prior art**

A need for lubricating oils which will remain serviceable for long periods of time at temperatures above 500° F. (260° C.) has long existed. The perfluoropolypropoxy polymers, i.e., polymers having the recurring group



and which are end-capped with perfluoroalkyl groups have been found to approach the desired performance characteristics stated above. By fractionation, oily fractions of such polymers are obtained which are operable as lubricating oils at temperatures as high as 800° F. (427° C.). Such oils have no apparent effect on metals and do not evidence degradation at temperatures up to about 400° F. (204° C.); however, at temperatures above 500° F. (260° C.), both metal corrosion and degradation of the oil occur. Representative metals which have been shown to corrode with such oils include steel, stainless steel, aluminum, titanium and titanium alloys. Accordingly, it is desirable, and it is one object of this invention, to provide these oils with an additive which eliminates or reduces both metal corrosion and oil degradation at extremely high temperatures; e.g., from 500° F. to 700° F. (371° C.).

To perform as an acceptable additive, the additive must have additionally acceptable properties over and above the properties of retarding corrosion and degradation. The additive must be compatible with the oil and have little, if any, effect on the lubricating properties of the oil, such as its lubricity, viscosity and viscosity index. It is another object of this invention to provide such a compatible additive. In addition, the additive must be soluble in the oil to an extent which produces an effective concentration for its purpose. The solubility

2

must be such that the additive will not separate from the oil, either at high operating temperatures or at low (ambient) storage or non-operating temperatures. The additive must also possess a high degree of thermal stability itself. It is still another object of this invention to provide an additive which possesses such desirable solubility and thermal properties with the perfluoropolypropoxy oils.

**SUMMARY OF THE INVENTION**

The novel compositions of this invention are perfluorinated polyether oil compositions comprising:

(a) A perfluorinated polyether oil selected from the class consisting of oils of the structure



and



wherein  $R_f$  is perfluoroalkyl of 1 through 6 carbon atoms,  $R'_f$  is perfluoroalkyl of 1 through 2 carbons and  $n$  is an integer denoting the degree of polymerization; said oil having an average molecular weight of at least 3000, a pour point of less than 10° C., and a maximum volatility of less than 50% at 204.4° C.; and

(b) An effective amount of a substituted guanamine of the structure



wherein  $R_f$  is defined as above and  $m$  is an integer of 0 through 100.

**DETAILED DESCRIPTION OF THE INVENTION**

**(A) The perfluorinated polyether oils**

The base oils employed in the compositions of this invention are perfluorinated polyethers which may be derived from hexafluoropropylene oxide. These oils are prepared by first polymerizing hexafluoropropylene oxide, either alone or in the presence of a carbonyl fluoride, a perfluoro acid fluoride or a perfluoro ketone, using certain fluoride ion containing catalysts or charcoal as taught by Moore et al. in U.S. Pat. 3,250,808, by Moore in Canadian Pat. 707,359, by Fritz et al. in U.S. Pat. 3,250,807, by Moore in Canadian Pat. 707,361, and U.S. Pat. 3,322,826 and by Selman in U.S. Pat. 3,274,239 to obtain hexafluoropropylene oxide polymers of the structure:



where  $R_f$  is a perfluoroalkyl group and  $n$  ranges from 0 to 100. These polymers are readily hydrolyzed in the presence of water to the corresponding acids of the structure:



These acids are converted to perfluorinated polyethers by reaction with elemental fluorine according to the proce-

dure of Miller in U.S. Pat. 3,242,218 to give products of the structure:



These polymers may also be converted to perfluorinated polyethers by ultraviolet light coupling with the elimination of the COF group as taught by Milian U.S. Pat. 3,214,478 to form oils of the structure:



The hexafluoropropylene oxide polymers may also be converted to products containing a single hydrogen of the structure:



as taught by Selman et al. in U.S. Pat. 3,342,875, but the presence of the hydrogen causes the resulting oils to be less desirable than those derived from the perfluorinated ethers.

Alternatively, as taught by Sianesi et al. in French Pat. 1,434,537, perfluorinated polyethers exemplified by the structures,



or



may be prepared from perfluoropropylene. Such materials may be converted to useful perfluorinated polyether oils by one or more of the methods for end-capping in the patent references mentioned above in this section. Thus it is seen that  $n$  in the oils employed herein is preferably between 1 and 100.

As indicated above, the perfluorinated polyether polymers may vary from low molecular weight products to very high molecular weight products. To be useful in the present invention, the perfluorinated polyesters must be chosen from this broader class of compounds to meet the requirements of volatility and pour point which are necessary to obtain useful oils. The oils must have a maximum volatility of 50% at 204.4° C. (400° F.) as determined by Federal Test Method FTMS-791, Method 351 and a maximum pour point of 10° C. (50° F.) as determined by ASTM-D-97. Within this class it has been found that oils having molecular weights of 3000 to 13,000 are preferable. Of course, the polymerization methods give mixtures of products so that the molecular weights are an average. Although a pure product having a specific molecular weight may be used, mixtures of products are equally useful if the variation in molecular weight is not too large. Usually, the most volatile lower molecular weight materials are removed from oils before use.

Oils having volatilities greater than that specified above are not useful because they do not have the service life required. Oils having pour points greater than 10° C. are not useful because, under many startup conditions, they would be too thick to provide lubrication before equipment in which the oils are being used had heated sufficiently to permit adequate oil flow to contacting metal surfaces.

Particularly preferred oils have the structure,



where  $R_f$  is a perfluoroalkyl group of from 1 to about 4 carbons, and which have a molecular weight range of from about 4500 to about 7000, and pour points of from about -10 to about -40° C.

#### (B) The substituted guanamine additives

The preparation of the substituted guanamines used as additives, with the structure shown above, comprises reacting an ester of the structure



where  $m$  is 0 to 100,  $R_f$  is  $C_{1-6}$  perfluoroalkyl and  $R$  is a lower alkyl, e.g., a methyl or ethyl group, with biguanide

under alkaline catalysis. This preparation is more fully described in applicants assignee's copending application, Ser. No. 734,546, filed concurrently herewith.

These substituted guanamines are used in an effective amount in the perfluorinated polyether oils. By "effective amount" is meant the amount required to produce useful inhibition of metal corrosion and oil degradation for the required service life of the device containing the oil at the desired operating temperature. Various metals differ considerably in the amount of corrosion which will occur and in promoting effect on oil degradation. Thus, the effective amount of additive will vary with the service and with the metals in contact with the oils.

In general the amount of the substituted guanamines required will be in the range of from about 0.1% by weight of the oil to about 8% by weight. At less than 0.1% concentration there is seldom enough additive to perform effectively. Additive concentrations above 8% seldom produce any increase in effectiveness. For a general purpose high-temperature oil it is usually preferable to add between about 2% and about 6% by weight of the substituted guanamines. This range provides for the vast majority of the needs for the oils.

Most preferably, the substituted guanamines are those in which  $m$  is an integer of 3 through 30.

The compositions of this invention are prepared by simply mixing the substituted guanamine with the perfluorinated polyether oil in the selected amounts.

#### (C) Examples

The following examples, illustrating the novel compositions of the invention and their effectiveness, are given without any intention that the invention be limited thereto. All percentages are by weight.

Compositions of this invention were tested using a modified form of the apparatus specified in the WADD Microoxidation-Corrosion Test of High Temperature Fluids, Fluids and Greases Section, Aeronautical Systems, Wright-Patterson Air Force Base, replacing the specified Pyrex tube with an Inconel tube. Basically the apparatus consists of a 3.18 mm. diameter Inconel tube adapted for mounting three washers outside the lower end. The 3.18 mm. tube is inserted inside a 20.6 diameter vertical Inconel tube so that the washers are immersed in a body of oil contained in the larger tube. The larger tube, which is adapted with a condenser for recovering any oil which may be stripped from the tube, is inserted in an aluminum heating block.

Various metal washers of the compositions in the following Table I were tested:

TABLE I

| Metal in washers                  | Composition                                                  |
|-----------------------------------|--------------------------------------------------------------|
| Group A. Titanium alloys:         |                                                              |
| Ti (6Al-4V)                       | 6% Al, 4% V; balance Ti.                                     |
| Ti (4Al-4Mn)                      | 4% Al, 4% Mn; balance Ti.                                    |
| Ti (A-70)                         | Essentially Ti.                                              |
| Group B. Ferrous alloys (steels): |                                                              |
| 410                               | 0.15% C, 12% Cr, 1% Mn, 1% Si.                               |
| 440C                              | 1.1% C, 17% Cr, 1% Mn, 1% Si, 0.75% Mo; balance Fe.          |
| M-2                               | 4% Cr, 2% V, 6.3% W, 5% Mo; balance Fe.                      |
| 52100                             | 1% C, 1.4% Cr, 0.3% Mn, 0.2% Si; balance Fe.                 |
| 4140                              | 0.4% C, 0.9% Cr, 0.9% Mn, 0.3% Si, 0.2% Mo; balance Fe.      |
| M-50                              | 0.8% C, 4% Cr, 0.25% Si, 4.5% Mo, 0.1% Ni, 1% V; balance Fe. |

The test consisted of placing test washers of the metals to be tested in the apparatus, adding sufficient oil composition to insure that the washers are covered, assembling the remaining apparatus and inserting it in the heating block. The oil is then heated to the test temperature and air is passed down through the smaller tube into the body of oil containing the washers. Test duration was 72 hours. Air flow rate into the oil during the test was 5 liters per hour, measured at 25° C.

Degradation in a test oil is evaluated by determining percent change in the viscosity of the test oil during the test. The results are expressed as:

Percent viscosity change

$$= \frac{cs \text{ after test} - cs \text{ before test}}{cs \text{ before test}} \times 100$$

where  $cs$  is the kinematic viscosity, at  $37.78^{\circ}\text{C}$ , in

inated substituent side chain of the substituted guanamine additives:



TABLE II.—OIL DEGRADATION AT SELECTED TEMPERATURES

| Example No. | m  | Metal                     | Wt. percent additive present | 72 hour fluid loss and viscosity change |                                    |                              |                                    |
|-------------|----|---------------------------|------------------------------|-----------------------------------------|------------------------------------|------------------------------|------------------------------------|
|             |    |                           |                              | 315.6° C. percent fluid loss            | (600° F.) percent viscosity change | 343.3° C. percent fluid loss | (650° F.) percent viscosity change |
| 1.          |    |                           | 0                            | 12.2                                    | -50.2                              | 79.7                         | -99.0                              |
| 2.          | 13 | A <sup>1</sup>            | 1.5                          |                                         |                                    | 9.0                          | -31.2                              |
| 3.          | 13 |                           | 2.8                          | 2.5                                     | +7.6                               | 3.2                          | +7.1                               |
| 4.          | 13 |                           | 5.8                          | 2.2                                     | +8.0                               |                              |                                    |
| 5.          | 20 |                           | 5.7                          |                                         |                                    | 5.1                          | +1.5                               |
| 6.          | 13 |                           | 0                            | 2.2                                     | -0.02                              | 6.2                          | -9.2                               |
| 7.          | 13 | B <sup>2</sup>            | 0.8                          |                                         |                                    | 1.0                          | +4.2                               |
| 8.          | 13 |                           | 2.8                          | 1.2                                     | +2.3                               | 0.9                          | +4.2                               |
| 9.          | 13 |                           | 5.8                          | 1.9                                     | +5.5                               |                              |                                    |
| 10.         | 20 |                           | 5.7                          | 0.88                                    | +7.8                               |                              |                                    |
| 11.         |    | Ti (6Al, 4V) <sup>3</sup> | 0                            | 22.0                                    | -53.6                              |                              |                                    |
| 12.         | 4  | Ti (6Al, 4V) <sup>3</sup> | 4.3                          | 8.5                                     | +12.6                              |                              |                                    |

<sup>1</sup> The A group of Table I tested together.

<sup>2</sup> The B group of Table I tested together.

<sup>3</sup> All washers in these test were Ti (6Al, 4V).

centistokes. When the sign of the percent viscosity change is negative, oil degradation is indicated. When the sign is positive, high temperature loss of volatile oil compo-

The data in Table II shows the effectiveness of the substituted guanamines in reducing oil degradation at  $315.6^{\circ}\text{C}$ . and at  $343.3^{\circ}\text{C}$ . respectively.

TABLE III.—CORROSION INHIBITION

| Example No. | m  | Metal         | Wt. percent additive present | 315.6° C. |          | 343.3° C. |          |
|-------------|----|---------------|------------------------------|-----------|----------|-----------|----------|
|             |    |               |                              | Control   | Additive | Control   | Additive |
| 13.         | 13 | Ti (6Al, 4V)  | 1.5                          |           |          | -0.03     | -0.07    |
| 14.         | 13 | Ti (6Al, 4V)  | 2.8                          | +0.04     | +0.04    | -0.03     | +0.09    |
| 15.         | 13 | Ti (6Al, 4V)  | 5.8                          | +0.04     | +0.05    |           |          |
| 16.         | 20 | Ti (6Al, 4V)  | 5.7                          |           |          | -0.03     | +0.01    |
| 17.         | 13 | Ti (4Al, 4Mn) | 1.5                          |           |          | -0.63     | -0.24    |
| 18.         | 13 | Ti (4Al, 4Mn) | 2.9                          | -0.19     | +0.01    | -0.63     | +0.10    |
| 19.         | 13 | Ti (4Al, 4Mn) | 5.8                          | -0.19     | +0.04    |           |          |
| 20.         | 20 | Ti (4Al, 4Mn) | 5.7                          |           |          | -0.63     | +0.18    |
| 21.         | 13 | Ti (A-70)     | 1.5                          |           |          | -0.29     | -0.20    |
| 22.         | 13 | Ti (A-70)     | 2.8                          | -0.10     | +0.04    | -0.29     | +0.21    |
| 23.         | 13 | Ti (A-70)     | 5.8                          | -0.10     | +0.04    |           |          |
| 24.         | 20 | Ti (A-70)     | 5.7                          |           |          | -0.29     | 0.04     |
| 25.         | 13 | 410           | 0.8                          |           |          | -1.32     | +0.01    |
| 26.         | 13 | 410           | 2.8                          | +0.04     | +0.01    | -1.32     | +0.03    |
| 27.         | 13 | 440C          | 0.8                          |           |          | -3.22     | +0.10    |
| 28.         | 13 | 440C          | 2.8                          | +0.21     | 0.00     | -3.22     | +0.13    |
| 29.         | 13 | M-2           | 0.8                          |           |          | -3.71     | +1.12    |
| 30.         | 13 | M-2           | 2.8                          | +0.33     | +0.03    | -3.71     | +0.17    |

nents is indicated. It will be noted in the following Table II that oil degradation is frequently accompanied by increased fluid loss from the apparatus. Degradation of polymer chains provides fragments having greater volatility than the original polymer.

Corrosion is determined by weighing the test washers before and after the test. Corrosion rate is calculated from weight change and known washer surface area. Before weighing, both before and after the test, the test washers are cleaned by scrubbing with scouring powder and water, rinsed with water, degreased and dried with acetone. The oil used in the following 30 examples has the structure:



where  $n$  is sufficiently large to afford an oil with an average molecular weight of about 5000.

In the following Tables II and III the letter  $m$  refers to the average degree of polymerization in the perfluor-

The data in Examples 13 to 30 of Table III demonstrate the effectiveness of the additives in reducing or preventing corrosion of titanium, titanium alloys, and ferrous alloys. Additive effectiveness is particularly marked at the higher of the two test temperatures. The other steels of Table I, 52100, 4140 and M-50 show little or no corrosion at  $315.6^{\circ}\text{C}$ . and at  $343.3^{\circ}\text{C}$ .

Similar results may be obtained with oils of the structure



or



The preceding representative examples may be varied within the scope of the present total specification disclosure, as understood and practiced by one skilled in the art, to achieve essentially the same results.

The foregoing detailed description has been given for clearness of understanding only and no unnecessary limi-

tations are to be understood therefrom. The invention is not limited to the exact details shown and described, for obvious modifications will occur to those skilled in the art.

The embodiments of the invention in which an exclusive property or privilege is claimed are defined as follows:

1. A perfluorinated polyether oil composition comprising

(a) a perfluorinated polyether oil selected from the class consisting of oils of the structure



and



wherein  $R_f$  is perfluoroalkyl of 1 through 6 carbon atoms,  $R'_f$  is perfluoroalkyl of 1 through 2 carbons and  $n$  is an integer denoting the degree of polymerization; said oil having an average molecular weight of at least 3000, a pour point of less than 10° C., and a maximum volatility of less than 50% at 204.4° C.; and

(b) a substituted guanamine of the structure



wherein  $R_f$  is defined as above and  $m$  is an integer of 0 through 100 present in an amount effective for corrosion inhibition and stabilization.

2. The composition of claim 1 wherein the substituted guanamine is present in an amount of between about 0.1 to about 8 percent by weight of the perfluorinated polyether oil.

3. The composition of claim 2 wherein the perfluorinated polyether oil has the structure



10 wherein  $R_f$  is perfluoroalkyl of 1 through 6 carbon atoms,  $R'_f$  is perfluoroalkyl of 1 through 2 carbon atoms; and  $n$  is an integer of between 1 and 100.

4. The composition of claim 3 wherein  $R'_f$  is 15  $-CF_2CF_3$ .

5. The composition of claim 4 wherein  $R_f$  is



and the oil has an average molecular weight of between 20 about 4500 and 7000.

20 6. The composition of claim 5 wherein  $m$  in the substituted guanamine is an integer of 3 through 30, and wherein the substituted guanamine is present in an amount of between about 2 to about 6 percent by weight of the perfluorinated polyether oil.

#### References Cited

##### UNITED STATES PATENTS

- |    |           |        |                 |       |          |
|----|-----------|--------|-----------------|-------|----------|
| 30 | 2,680,717 | 6/1954 | Little          | ----- | 252—51 X |
|    | 3,306,854 | 2/1967 | Gumprecht       | ----- | 252—49.9 |
|    | 3,453,275 | 7/1969 | Grindahl et al. | ----- | 252—51 X |

DANIEL E. WYMAN, Primary Examiner

W. J. SHINE, Assistant Examiner

35 U.S. Cl. X.R.

252—392, 403